

# UNITED STATES PATENT OFFICE.

FREDRICK C. DONOVAN, OF VANCOUVER, BRITISH COLUMBIA, CANADA.

## COMPOSITION OF MATTER FOR CLEANING AND POLISHING PAINTED OR VARNISHED SURFACES.

1,123,709.

Specification of Letters Patent.

Patented Jan. 5, 1915.

No Drawing.

Application filed March 25, 1913. Serial No. 756,808.

*To all whom it may concern:*

Be it known that I, FREDRICK C. DONOVAN, a subject of the King of Great Britain, residing at Vancouver, in the Province of

5 British Columbia, Dominion of Canada, have invented a new and useful Composition of Matter for Cleaning and Polishing Painted or Varnished Surfaces, of which the following is a specification.

10 My invention relates to polishes and cleaners and has for its object the production of a composition of matter which will resurface and renew paints, varnishes, and enamels, such as are commonly used on 15 automobiles, furniture, interiors, and the like. Such surfaces, and particularly automobile, are exposed to the action of the elements, and are sometimes cleaned with acids or alkalis. All of this tends to dull 20 the luster of the finished surface and renders the objects unsightly. These surfaces are originally produced by the repeated applications of thin coats of filler or varnish, these coats being repeatedly rubbed 25 down with pumice stone or the like. When they become dulled by use it is common practice to add subsequent coats which is not entirely satisfactory as to results, and which is expensive and requires a consider- 30 able time.

With my invention I resurface and renew the original finish at a fraction of the expense and in a fraction of the time required for repainting and revarnishing.

35 My compound consists of a polishing material, such as tripoli or the like, carried in a suitable vehicle, such as linseed oil, together with a solvent such as turpentine. For the purpose of filling cracks in the sur- 40 face a small amount of shellac dissolved in alcohol may be used.

I find that tripoli is a very satisfactory polishing material but other similar materials may be used if desired. In the same 45 manner, while I use boiled linseed oil, there are a number of similar materials, which give good results. While I use turpentine there are other solvents used by painters which give nearly as good results, and while 50 I prefer pure shellac gum mixed with alcohol as my fourth ingredient this may be left out or a similar gum may be used.

While I give in this specification a preferred formula I wish the doctrine of equivalents to be broadly applied as briefly outlined 55 above.

My invention therefore consists broadly of a composition comprising a polishing material, a vehicle, and a solvent with or without a gum. A preferred form is made 60 up as follows: boiled linseed oil 3 gallons, spirits of turpentine 2 gallons, tripoli 8 ounces, shellac dissolved in spirits 4 ounces. The proportions of this mixture may be considerably varied without affecting its 65 efficiency and the above is given merely as a formula that I have found to work well in practice.

The method of operation in cleaning any 70 object, for example, an automobile, using my composition of matter is as follows: A piece of soft cheese cloth or old turkish toweling is saturated with water and a small amount of water is thrown upon the surface to be cleaned. A small portion of the composition is then put upon the cloth and the surface is rubbed therewith. No preliminary washing is necessary. The various ingredients form an emulsion which takes a 75 pasty form, the vehicle and the solvent loosening the grease and dirt which is also cut by the polishing material. The polishing material acts upon the roughened surface of the old paint giving it a high polish. After 80 going over the surface it is washed with clear water, without soap, and the surface is left in a hard highly polished condition. I 85 have found that even on new automobiles that have never been used or washed that my composition of matter greatly enhances 90 the polish and I have repeatedly so applied it.

The small portion of shellac that I use 95 serves to fill up minor scratches and indentations and to give a thin film of new material over the entire surface treated.

My invention should not be confused with either soaps or the so-called furniture polishes. In the former it is almost impossible to produce a composition that is not alkaline 100 and the action is that of a soap. On the other hand furniture polishes are generally strongly acid. Either acids or alkalis have a destructive action on highly polished sur-

faces and my composition of matter which is entirely neutral is absolutely harmless to such surfaces.

I claim as my invention:

- 5 1. A composition of matter in the form of a liquid adapted to form an emulsion with water comprising a polishing abrasive, a neutral vehicle for said abrasive, and a solvent, substantially in the proportions de-  
10 scribed.
2. A composition of matter in the form of a liquid adapted to form an emulsion with water comprising a polishing abrasive, a neutral vehicle for said abrasive, a small  
15 portion of resinous gum dissolved in alcohol, and a solvent, substantially in the propor-  
tions described.
3. A composition of matter in the form of a liquid adapted to form an emulsion with  
20 water, comprising tripoli, boiled linseed oil, and spirits of turpentine, substantially in the proportions described.
4. A composition of matter in the form of a liquid adapted to form an emulsion with  
25 water, comprising tripoli, a small portion of

resinous gum dissolved in alcohol, boiled linseed oil, and spirits of turpentine substan-  
tially in the proportions described.

5. A composition of matter for cleaning and polishing painted, varnished, or enam-  
30 eled surfaces, comprising tripoli, eight  
ounces; boiled linseed oil, three gallons; and  
spirits of turpentine, two gallons.

6. A composition of matter for cleaning and polishing painted, varnished, or enam-  
35 eled surfaces, comprising tripoli, eight  
ounces; boiled linseed oil, three gallons;  
spirits of turpentine, two gallons; and shel-  
lac in alcohol, four ounces.

7. A composition of matter in the form 40  
of a liquid adapted to form an emulsion with water, comprising tripoli, shellac in  
alcohol, boiled linseed oil, and spirits of tur-  
pentine, substantially in the proportions de-  
scribed.

FREDRICK C. DONOVAN.

Witnesses:

FRED P. GORIN,  
R. SMALLEY.